

Patented Apr. 8, 1924.

1,489,429

## UNITED STATES PATENT OFFICE.

BERTON H. DE LONG, OF SPRINGMONT, SINKING SPRING, AND FRANK R. PALMER, OF READING, PENNSYLVANIA, ASSIGNEES TO THE CARPENTER STEEL COMPANY, OF READING, PENNSYLVANIA, A CORPORATION OF NEW JERSEY.

### CHROMIUM-STEEL ALLOY.

No Drawing.

Application filed August 6, 1921. Serial No. 490,383.

To all whom it may concern:

Be it known that we, BERTON H. DE LONG and FRANK R. PALMER, citizens of the United States, residing, respectively, at 5 Springmont, Sinking Spring P. O., and Reading, in the county of Berks and State of Pennsylvania, have invented certain new and useful Improvements in Chromium-Steel Alloys, of which the following is a 10 specification.

Our invention relates to steel alloys characterized by a considerable chromium content, and the main object is to provide for securing the maximum of known advantages incident to the use of chromium while at the same time eliminating or reducing known disadvantages and giving added desirable quality to the product. To this end the invention consists essentially in employing copper as an alloy element in connection with the chromium and with carbon, as fully set forth hereinafter and clearly defined in the claims.

The type analysis of our improved alloy, 25 as most satisfactorily tested particularly for the purposes hereinafter specifically referred to, may be stated as follows; it being understood that the ferrous base employed may be of any ordinary commercial 30 content without essentially affecting the results attained; to wit:

|          |        |
|----------|--------|
| Carbon   | 4.0%   |
| Chromium | 20.00% |
| Copper   | 1.00%  |

In our further combined use of the alloying elements above noted, we have discovered that the proportions stated as typical may be varied, with corresponding variation of the characteristic results in all cases secured, within the following limits, 40 to wit:

Carbon, from .05% to 3.50%.

Chromium, from 8.00% to 60.00%.

45 Copper, from .50% to 10.00%.

The desirability of a non-corrosive or corrosion-resisting alloy steel is well understood; and the effects of chromium in this direction have been recognized, and said 50 element used in different proportions and in connection with carbon, particularly for a hardened product adapted for cutlery and

other cutting tools. The use of large percentages of chromium however have been attended by well known incidental disadvantages, and the carbon content tends to impair the surface resistance to deterioration attainment of which is the main purpose we have in view. We have discovered that the employment of copper as stated, in connection with these elements, enables the overcoming of the disadvantages otherwise incident to desired use of the chromium and carbon elements, and particularly that it enables the production of a readily malleable alloy having high surface resistance to corrosion or deterioration irrespective of hardening of the surface, and of desired uniform texture and quality. The percentage of copper employed, relative to the percentages of chromium and carbon and of the ferrous base, may be varied within the limits above stated, with substantial attainment of the desired non-corrosive effect and corresponding variations in specific structure and quality; approximately the relative proportions definitely stated above however having been found most satisfactory for ordinary uses of an unhardened forgeable and corrosion-resisting alloy steel, though the essential corrosion-resisting quality is desirably imparted by the copper element within a range of constituent elements which would exclude the forgeable quality specifically provided for.

What we claim is:

1. A corrosion-resisting article of manufacture composed of a ferrous alloy containing chromium between eight per cent (8%) and sixty per cent (60%), carbon not in excess of three and one-half per cent (3.5%), and between one-half per cent (.5%) and ten per cent (10%) of copper.

2. A corrosion-resisting article of manufacture composed of malleable ferrous alloy containing approximately twenty per cent (20%) of chromium, four tenths per cent (.40%) of carbon, and one per cent (1%) of copper.

In testimony whereof we affix our signatures.

BERTON H. DE LONG.  
FRANK R. PALMER.